

April 16, 1963

M. TANENBAUM

3,085,981

FERRIMAGNETIC CRYSTALS

Filed March 25, 1960

FIG. 1



FIG. 2



FIG. 3



FIG. 4



FIG. 5



INVENTOR  
M. TANENBAUM  
BY  
George S. Radig  
ATTORNEY

# United States Patent Office

3,085,981

Patented Apr. 16, 1963

1

3,085,981

## FERRIMAGNETIC CRYSTALS

Morris Tanenbaum, Madison, N.J., assignor to Bell Telephone Laboratories, Incorporated, New York, N.Y., a corporation of New York

Filed Mar. 25, 1960, Ser. No. 17,539  
1 Claim. (Cl. 252—62.5)

This invention relates to an improved ferrimagnetic structure, particularly in ferrimagnetic garnets. More specifically, it relates to a structure wherein the demagnetizing effects on the crystal surface are minimized.

With the advent of more perfect crystal growing techniques, particularly with respect to ferrimagnetic garnets, superior resonance characteristics have been found to depend more and more on the surface characteristics of the crystals. Heretofore, with conventional ferrites, the crystals possessed interior faults which themselves limited the resonance character so that a high degree of smoothness was not necessary.

It has been found that the garnet structures being grown today are of such quality that the resonance characteristics, for instance, the resonance line width, are limited by the degree of surface smoothness. Considering a perfect sphere of single crystal yttrium-iron garnet, the relations between the frequency  $v$  for resonance and the direct-current magnetic field  $H$  for such a sphere is given by the following equation:

$$v = .446 H$$

where  $v$  is in megacycles per second and  $H$  is in oersteds. The line width of the resonance expressed by the change in magnetic field required for the absorption to fall to one-half of its maximum value will be a few tenths of an oersted at room temperature. Such narrow line widths have been observed in single crystals of yttrium-iron garnet at frequencies in the neighborhood of 5,000 megacycles per second. However, these narrow ideal lines can only be obtained by the most careful polishing of the small spheres. These spheres are generally about 15 mils in the diameter and must be polished approximately one week with successive grades of abrasive material until they achieve a sphericity and surface finish which is adequate. Even after this laborious and expensive polishing, careful examination of the surface of these spheres indicates that small pits and scratches still exist and are contributing to the measured resonance line width. These effects occur because of the demagnetizing fields which are produced when the arrays of magnetic dipoles in the sphere reach an abrupt discontinuity at the imperfect surface. Typical resonance line widths of garnets before and after various grades of polishing have been studied by Spencer, LeCraw and Porter and are reported at pages 1311 through 1313, "The Physical Review," volume 110, No. 6, June 15, 1958.

The theory and measurement of resonance line widths can be found in "Ferrites" by J. Smit and H. P. J. Wijn.

An object of the present invention, therefore, is to provide a crystal structure in which the demagnetizing effects of minute surface imperfections, left even as a result of extensive physical polishing, are rendered less effective.

The present invention proposes to diffuse into the outer surface of the crystal a nonmagnetic ion which will substitute for the iron ion in the garnet lattice. The resulting crystal will then have an outer shell region of nonmagnetic garnet structure with a ferrimagnetic interior region. The interface between these regions exhibits a continuity or smoothness far superior to that of the original surface.

This may perhaps be best understood when considered in conjunction with the drawing in which:

2

FIG. 1 is a sectional view of a portion of a typical garnet crystal having surface characteristics after rough polishing;

5 FIG. 2 is a sectional view of a portion of the same crystal during the first phase of the treatment of the invention;

FIG. 3 is a sectional view of a portion of the same crystal at a subsequent stage of the operation;

10 FIG. 4 is a sectional view of a portion of the desired finished crystal; and

FIG. 5 is a schematic view of an appropriate apparatus used in obtaining the desired crystal.

Referring to FIGS. 1 through 4 which show the crystal in various stages of treatment according to the invention, 15 numeral 1 refers to the ferrimagnetic interior layer and 2 denotes the crystal surface. FIGS. 2 through 4 show the diffusion layer of nonmagnetic material 3, and the interface between the magnetic and nonmagnetic regions 4.

The critical interface ordinarily impairing the resonant 20 properties is the ferrimagnetic surface denoted 2 in FIG. 1. In FIGS. 2 through 4 the original crystal surface 2 is now nonmagnetic and the irregularities there will not affect the magnetic dipoles. The critical interface then becomes interface 4, that is, the interface between the 25 magnetic and nonmagnetic regions. As is seen, this diffusion layer interface, that is, the interface between the magnetic region 1 and the nonmagnetic region 3 will initially reflect the surface imperfections. However, the deeper the layer diffuses between preferred depths of 30 1-50 microns depending upon the depth of the initial irregularities, the less pronounced these irregularities become. This is apparent from an examination of the changing character of the interface 4 in FIGS. 2 through 4.

FIG. 4 then shows the finished crystal 15 mils in diameter having an appropriate diffusion layer of the order of 15 microns. The interface there appears substantially smooth. Hence, the magnetic dipoles leaving the ferrimagnetic region will emerge through the spherical surface having a smoothness which will not significantly 35 upset their resonance properties.

The diffusion procedure makes use of an oxide source of a group 3 metal, typically Ga or Al. The group 3 metal upon diffusing into the iron garnet replaces the magnetic iron ion in the lattice forming a nonmagnetic garnet such as  $Y_3Ga_5O_{12}$ . The source is conveniently a mixture of the group 3 metal oxide and the free group 3 metal. These materials react to form a suboxide of the group 3 metal which is sufficiently volatile and readily diffuses into the iron garnet placed adjacent the source. 40 With respect to gallium the reactions appear thus:



55 The following specific embodiment is given to illustrate one particular procedure for practicing the invention. The apparatus used is a typical two-zone furnace as is well known in the art and shown schematically in FIG. 5. A quartz tube 11 is evacuated to approximately  $10^{-5}$  millimeters of mercury. A mixture of 1 gram of powdered gallium oxide is intimately mixed with 2 grams gallium metal, the metal being liquid at room temperature, and the mixture, contained in the silica boat 12, is placed in the first zone 13. This zone, heated by coil 14 which controls the atmosphere over the  $\text{Ga}, \text{Ga}_2\text{O}_3$  system, is heated to 700° C. A ferrimagnetic garnet crystal was coarsely polished with an abrasive of 3 microns mean grit size and consequently exhibited surface characteristics similar to those of FIG. 1, having an average depth of 3 microns. The crystal 15, 15 mils in di-

ameter and having the composition  $Y_3Fe_5O_{12}$ , is placed in the tube at zone 16. The garnet before treatment has a resonance line width of approximately 2 oersteds. The zone 16, controlled thermally by coil 17, is heated to 1200° C. These conditions are maintained for a period of 24 hours. This two-zone diffusion technique is known to the art and is treated by Frosch and Derrick in the "Journal of the Electrochemical Society," volume 105, December 1958, at pages 695 through 699.

Upon completion of the required period, the garnet crystal exhibits a diffusion layer of nonmagnetic material to a depth of approximately 15 microns and shows an interface between the non-magnetic diffused layer and the remaining ferrimagnetic portions of the crystal which has a greater degree of uniformity than the surface of the crystal. This smoother interface is shown in the cross-section of FIG. 4. The resonance line width of this crystal after treatment according to the invention is .4 oersteds or a reduction by a factor of 5.

This procedure is given as exemplary only and is not intended as limiting the invention. Hence, any ferrimagnetic garnet may be so treated to reduce the adverse ferrimagnetic effects of surface imperfections. These encompass yttrium-iron garnets and rare earth iron garnets. The nonmagnetic ion to be diffused into the garnet lattice is restricted by the size of the atom. Gallium and aluminum are appropriate.

The process conditions vary according to the materials

and systems employed, but generally, temperatures between 500° C. and 1000° C. in zone 1 and 900° C. to 1500° C. in zone 2 are proper. The atmosphere in the quartz tube is preferably a vacuum. Alternatively, an inert atmosphere such as argon gas may be used. While the invention has been described in terms of spherical crystals it is obvious to one skilled in the art that various other shapes such as rods or disks may be advantageously treated in this manner.

What is claimed is:

The method of treating a single crystal yttrium iron garnet to provide a smooth magnetic surface which comprises diffusing into the surface of said garnet an ion selected from the group consisting of aluminum and gallium whereby the diffusion layer is rendered non-magnetic and the ferrimagnetic surface exhibits a greater degree of uniformity than the surface of the garnet crystal.

#### References Cited in the file of this patent

#### UNITED STATES PATENTS

2,725,315      Fuller \_\_\_\_\_ Nov. 29, 1955  
2,947,923      Pardue \_\_\_\_\_ Aug. 2, 1960

#### OTHER REFERENCES

Pauthenet: Supplement to J. of Applied Physics, vol. 30, No. 4, pages 290S-292S, April 1959.